

June 9, 1953

C. V. LITTON

2,641,555

NONEMISSIVE ELECTRODE AND METHOD OF MAKING

Filed Jan. 18, 1950



INVENTOR  
CHARLES V. LITTON

BY  
Shawas Z. Leyden  
ATTORNEY

## UNITED STATES PATENT OFFICE

2,641,555

NONEMISSIVE ELECTRODE AND METHOD  
OF MAKING

Charles V. Litton, Redwood City, Calif.

Application January 18, 1950; Serial No. 139,186

2 Claims. (Cl. 117—46)

1

This invention relates generally to elements for use in electron discharge devices, and particularly to non-emissive electrodes which retain the non-emissivity even when used in conjunction with emitters bearing a coating of alkaline earth oxide.

It is well recognized that in an electron discharge device in which an electron stream moving from an emitter to an anode or collector is controlled by variation of the potential of an electrode interposed in or disposed nearby the electron stream, the control electrode may be emissive itself or it may become emissive under conditions of use unless certain precautions are taken in the manufacture of this electrode. This emissivity of the control electrode may be due either to normal emissivity resulting from heating of the electrode due to its close proximity to the hot emitter, especially in high power transmitting tubes used at high frequencies, or it may be due to secondary emissivity resulting from impingement of high speed electrons upon the control electrode. Irrespective of the cause of emission from the control electrode, it is obvious that such emission must be minimized, if not indeed entirely eliminated, if optimum tube operation is to be effected.

It is known that a vacuum tube electrode made of carbonized nickel is considerably superior to untreated nickel from the standpoint of non-emissivity because, when untreated nickel is utilized in conjunction with thermionically emissive cathodes, particularly cathodes coated with oxides of the alkaline earth metals, there is a tendency for the cathode coating material to 35 volatilize or disintegrate and deposit upon the other electrodes of the tube which, upon becoming heated, fail to perform their expected function and become emitters of electrons. When such electrodes are carbonized, however, the carbonized surface not only is itself non-emissive but also it inactivates material deposited on it from the cathode, thus preventing the emission of electrons but also increases the ability of the electrodes to radiate heat, thereby decreasing 45 their operating temperatures.

Non-emissive electrodes formed of carbonized nickel wires or strips have been found satisfactory when utilized in small tubes, but when attempts have been made to employ them in power tubes the nickel softens due to heating and tends to lose its shape, while in high-power tubes, especially tubes for use at high frequencies where the tube elements are in exceedingly close proximity, it completely loses its strength at the 50

operating temperatures of the tubes. In order to avoid this difficulty, it has been proposed to utilize other metals having a higher melting point than nickel, say above 1600° C., and a correspondingly high strength at the operating temperature of the tube, such as molybdenum, platinum, zirconium, tungsten or tantalum, but when attempts were made to carbonize such metals it was found that they became highly brittle and were unsuitable for use.

It is also known that a metal such as molybdenum or tungsten having a sufficiently high melting point so that its strength will be preserved at the operating temperature of the tube, when coated by any suitable method, such as by electrodeposition or spraying, with a metal that may be easily carbonized, such as nickel, cobalt, iron, or an alloy, such as nichrome, may not only be carbonized, but it is suitable as a material from which non-emissive electrodes for high-power electron tubes may be produced. However, it is found that the useful life of these electrodes is subject to wide variation, due perhaps to imperfections and nonuniformities of the metal coating that eventually permit migrations of carbon through the coating and into the underlying metal, resulting in impairment of the strength of said metal and removing the carbon coating from the electrode surface thus causing it to lose its non-emissivity.

The present invention is concerned with a method for producing a non-emissive electrode which, even if used at the elevated operating temperatures usual in tubes with a cathode having an alkaline earth oxide coating, remains substantially non-emissive under ordinary operating conditions.

Regarded in certain of its broader aspects, the novel non-emissive electrode according to the present invention comprises a refractory metal base shaped in the desired electrode form, bearing a coating produced by initially coating the metal base with at least one alkaline earth oxide, and thereafter heating the oxide coated base at a temperature at least equal to and preferably well above the temperature at which an alkaline earth oxide coated filament of a vacuum tube is normally operated in a carbonaceous atmosphere, as hereinafter defined, at a reduced pressure for a brief period of time. The electrode after being so processed is not only initially free of primary or secondary emission, even when operated at high temperatures in conjunction with an alkaline earth oxide coated emitter, but remains non-

emissive during use under ordinary operating conditions.

To facilitate a better understanding of the subject matter of this invention reference is made to the accompanying drawing which is a flow sheet correlating the steps in the manufacture of a vacuum tube embodying the principles of this invention.

It will be noted that the first step in the manufacture of a vacuum tube as represented in this flow sheet is the formation of the basic structure of the electrode from a refractory metal. This step in the procedure is in accordance with common practice in the vacuum tube manufacturing art and need not be described in detail except to mention that the refractory metal used is one that retains its physical integrity at high temperatures without melting, softening or bending, and which does not so persistently retain occluded gases as to present problems during the outgassing and evacuation of the tube. Among the refractory metals that have been found satisfactory for this purpose are tantalum, platinum, molybdenum and nickel, the last mentioned metal, because of its low melting point being useful primarily in types of tubes that are operated at elevated but not abnormally high temperatures.

After the refractory metal has been shaped into the form desired for the finished electrode, it is provided with a coating comprising at least one alkaline earth oxide selected from the class consisting of barium oxide, strontium oxide and calcium oxide. This coating may be applied by spraying, dipping, electrophoresis or by any of the other known methods that are commonly employed in vacuum tube manufacture to produce adherent, uniform and pit-free coatings of this type. It is also to be recognized that the invention may be practiced by producing the oxide coating as a result of heat treatment of an alkaline earth carbonate coating in well known manner after it has been applied to the electrode in any of the ways above mentioned.

In accordance with the present invention the next step in producing the non-emissive electrode is a brief heat treatment of the alkaline earth oxide coated refractory metal in a carbonaceous atmosphere, as hereinafter defined, under reduced i. e. sub-atmospheric, pressure and with the electrode at a temperature at least approximating and preferably substantially exceeding the normal operating temperature of an alkaline earth oxide coated filament in a vacuum tube, whereby the character of the coating is altered so that the coated electrode acquires its characteristic non-emissivity.

The term carbonaceous atmosphere as herein employed means an atmosphere containing vapor of a liquid hydrocarbon of the type described below which has low viscosity and surface tension such that it will readily penetrate the minute pores of the oxide coated electrode and further characterized in decomposing at the temperatures used in this process to yield carbon or a residue predominantly comprised of carbon. It will be understood that the term hydrocarbon as herein employed is not used in a limited sense of reference to oxygen-free carbon-hydrogen compounds but includes such oxygen-containing carbon-hydrogen compounds as esters, ethers, and the like that otherwise satisfy the physical requirements set forth above. Among the hydrocarbons that have been found suitable for this purpose are oils such as are used in oil diffusion pumps for instance the hydrocarbon

10  
5

oil known under the trade name "Octoil" which is dioctyl phthalate, an oily material having approximately the same viscosity as ordinary salad oil and a boiling point of about 122.5° C. at 10<sup>-2</sup> mm. "Pennzoil SAE 30," which is an automotive lubricant oil derived from paraffinic base Pennsylvania crude oil, may be used. It will be understood that these oils usually if not invariably contain oxygen either in dissolved elemental or in combined state.

15  
20

The concentration of the hydrocarbon in the carbonaceous atmosphere is not critical, although of course it will be obvious that the time of treatment in order to produce the desired result is related to the hydrocarbon concentration. However, satisfactory effects are produced if the hydrocarbon concentration is merely that resulting from the normal vapor pressure of the hydrocarbon i. e. that quantity of hydrocarbon in the atmosphere supernatant the liquid hydrocarbon under the operating condition aforesaid.

25  
30  
35

A procedure that has been found satisfactory according to the present invention for processing the alkaline earth oxide coated electrodes to convert the same to non-emissive electrodes involves the mounting of the oxide coated electrode in a vacuum chamber connected directly with an oil diffusion pump, using no means such as cold traps or charcoal for preventing normal back diffusion, and provided with means for heating the electrode to a high temperature. The oil in the diffusion pump is one of those above mentioned. Initially the electrode is "out-gassed" at about 900° C. for about 10 minutes at a pressure of 10<sup>-7</sup> mm. mercury, then the pressure is adjusted to 10<sup>-4</sup> to 10<sup>-3</sup> mm. mercury and the electrode is flashed at about 1300° C. for a period of 10 minutes or thereabouts, after which the emission of the electrode is measured at about 900° C. and 10<sup>-7</sup> mm. mercury pressure. If the electrode is found to be emissive, the preceding steps are repeated, although usually this is unnecessary. The foregoing procedure describes the treatment of a nickel base electrode but may be equally well applied to electrodes having a different higher melting point refractory metal base in which instance the flashing temperature used may be higher, for instance about 1600° C. for a platinum base electrode.

40  
45  
50

In the above described procedure the normal vapor pressure of the oil in the diffusion pump provides a sufficient quantity of carbonaceous component in the atmosphere to effect the subtle change in the oxide coating whereby it loses its normal emissivity and becomes permanently non-emissive. The precise manner in which this change occurs and the changes, if such occur, in the chemical composition of the oxide surface during the treatment in the carbonaceous atmosphere, are presently little understood, hence the necessity of defining the article in terms of the process for its manufacture. In connection with the reaction temperatures above set forth, it will be recognized that the temperatures stated are approximations within the experimental limitations imposed by difficulties in measuring such high temperatures. Also to be considered is the fact that the reaction between the carbonaceous atmosphere and the oxide coating on the metal is an exothermic reaction and thus there is at least a tendency for the initiation of the reaction to be reflected in a temperature rise independent

55  
60

70  
75

of the temperature to which the electrode is heated. When reference is made herein to the temperature at which an alkaline earth oxide coated filament is operated while in a vacuum tube, it will be understood that this type of filament is usually operated at about 850° to 900° C. In practicing the process according to this invention, however, it is desirable to use temperatures considerably higher than this, say about 1300° C., or even higher with those refractory metals of very high melting point.

When the oxide coated electrode has been processed as above described it is removed from the carbonaceous atmosphere of the chamber and it is then mounted in the usual manner within an envelope, together with the other tube elements and the alkaline earth oxide coated cathode, in the relationship that the various elements will occupy in the finished vacuum tube and, if desired, the assembly is then further processed according to known and usual techniques in vacuum tube manufacture. It is found that under conditions of use the control electrode so prepared permanently retains its characteristic non-emissivity under ordinary operating conditions.

Having thus described the subject matter of the present invention what it is desired to secure by Letters Patent is:

1. A method for making a non-emissive electrode for use in electron discharge devices comprising the steps of forming a base from a refractory metal element selected from the group of non-ferrous metallic elements having a boiling point of 2900 degrees C. or over, a 30 cubic lattice crystalline structure, and appearing

in the periodic table in group V or a higher group, consisting of tantalum, platinum, nickel and molybdenum; coating said base with an alkaline earth oxide, and heating the oxide electrode in an atmosphere of a hydrocarbon oil vapor that readily penetrates the pores of the oxide electrode at a temperature sufficient to decompose the hydrocarbon and leave a carbon residue.

- 10 2. A non-emissive electrode for use in an electron discharge device comprising a base of a metallic element selected from the group of refractory non-ferrous metallic elements having a boiling point of 2900 degrees C. or over, a cubic 15 lattice, crystalline structure, and appearing in the periodic table in group V or a higher numbered group, consisting of tantalum, platinum, nickel and molybdenum; an initial coating of alkaline earth oxide which has been heated in 20 an atmosphere of a hydrocarbon oil vapor that readily penetrates the pores of the oxide electrode at a temperature sufficient to decompose the hydrocarbon and leave a carbon residue.

CHARLES V. LITTON.

References Cited in the file of this patent

UNITED STATES PATENTS

| Number    | Name    | Date          |
|-----------|---------|---------------|
| 1,862,138 | Elsey   | June 7, 1932  |
| 1,880,937 | Elsey   | Oct. 4, 1932  |
| 1,897,933 | Guthrie | Feb. 14, 1933 |

FOREIGN PATENTS

| Number    | Country   | Date          |
|-----------|-----------|---------------|
| 23,525/35 | Australia | July 16, 1935 |